

# UNITED STATES PATENT OFFICE.

WILLIAM HOSKINS, OF LA GRANGE, ILLINOIS.

## SIZING COMPOSITION.

940,317.

No Drawing.

Specification of Letters Patent. Patented Nov. 16, 1909.

Application filed March 19, 1909. Serial No. 484,539.

To all whom it may concern:

Be it known that I, WILLIAM HOSKINS, a citizen of the United States, residing at La Grange, in the county of Cook and State of Illinois, have invented a new and useful Improvement in Sizing Compositions, of which the following is a specification.

My object is to provide, as a new article of manufacture, paper - sizing compounded in such a way as to render its use by paper manufacturers particularly convenient and economical and enable them, furthermore, to effect the results desired in the ultimate paper product with greater uniformity and less trouble than hitherto.

In the process of manufacturing paper, rosin-soap, called rosin-size, is added to the pulp during the beating operation and thoroughly mixed therewith. Alum, or aluminum sulfate, is then added to react with the rosin-soap and decompose and set free rosin and form aluminum resinate. Authorities differ as to the precise reactions that take place, but the effect upon the pulp is to cause a certain amount of the rosin, or aluminum resinate, to adhere to the particles of fiber, so that when the sheet of paper is made it is less pervious to water than would be the case without the sizing. The rosin-soap is ordinarily produced, at the paper mill, by heating the rosin in contact with a solution of soda ash, or caustic soda, by means of steam. To produce a good quality of sizing requires time, skill and care, and to effect the best results a knowledge of the purity of the constituents is necessary for the purpose of arriving at the correct proportions to be used and to avoid waste. Different lots of size will vary materially in the proportion of water present, and this leads to uncertainty as to the quantity of size to be added to the pulp, and also to the alum required, and this uncertainty tends toward inferiority and lack of uniformity in the final product and also to a waste of material. To avoid the above difficulties I provide a uniform sizing mixture so compounded as to produce the desired results in an unvarying manner.

In carrying out my invention I proceed as follows: To, say, 100 pounds of a certain lot of rosin I add approximately 11½ pounds of caustic soda, the precise amount necessary for any given lot of rosin being accurately determined by chemical test. I also add sufficient water, say, 25 per cent. of the weight

of the alkali, to cause ready saponification. These ingredients are thoroughly mixed together and heated, preferably in a steam-jacketed chamber, until saponification is complete. The mixture is then allowed to cool, becoming a brittle mass of rosin-soap, easily pulverized, and after its pulverization I mix with it, say, 50 pounds of an inert pulverulent material, such as china clay, or talc, to prevent the particles of the rosin-soap from adhering to each other and forming lumps, as would occur if moisture were absorbed thereby, or if its temperature were raised. To the dry pulverulent mixture thus produced, I prefer to add, say, 16.6 pounds of a dry and powdered rosin-soap-decomposing reagent, such, for example, as aluminum sulfate, incorporating it thoroughly with the other particles. I find that it is desirable to use as such reagent dehydrated alum (alum which has been deprived of its water of crystallization), as this dissolves in water much more slowly, even in a powdered state, than does the powdered rosin-soap, thus allowing time for the thorough mixing of the soap with the pulp before it is acted upon to any extent by the alum.

Dry rosin-soap when in lump form dissolves very slowly and when it is employed the practice is to liquefy it by heating in contact with water before adding it to pulp in order to mix therewith quickly and properly. If the rosin-soap is pulverized, however, and kept from agglomerating into lumps, as by having incorporated with it an inert material, such as powdered china clay, it dissolves quickly. China clay is frequently used as a constituent part of paper pulp, and the relatively small quantity of the same, or equivalent inert material, necessary for keeping the rosin-soap in a pulverized condition, would be of no disadvantage to the paper. Pulverized rosin-soap mixed with a suitable quantity of pulverized inert material may be provided without the decomposing reagent to paper manufacturers, who, after mixing it with pulp, could add thereto the desired quantity of alum or equivalent material. I believe, however, that, as a rule, a more uniform and desirable product would be obtained by paper manufacturers if the compound of pulverized rosin-soap (of known chemical composition) and inert material, has mixed therewith, in the first instance, only the necessary and most desirable quantity of soap-decom-

posing reagent, also of known analysis, thereby making it necessary to follow but the single rule of mixing a given quantity of the compound with a given amount of paper stock for certain results.

5 The compound may be provided in bags or other suitable packages and by its use little skill or judgment on the part of the operator is required for producing the desired results in paper manufacture.

10 What I claim as new and desire to secure by Letters Patent is—

15 1. A paper sizing compound, consisting of a mixture of saponified rosin, inert material and a rosin - soap - decomposing reagent, in suitable proportions, all the ingredients of the mixture being in dry, pulverulent condition, for the purpose set forth.

2. A paper sizing compound, consisting of a mixture of saponified rosin, inert material 20 and a rosin-soap-decomposing reagent more slowly soluble than rosin-soap, in suitable proportions, all the ingredients of the mixture being in dry, pulverulent condition, for the purpose set forth.

25 3. A paper sizing compound, consisting of a mixture of saponified rosin, inert material, dehydrated alum or aluminum sulfate, in suitable proportions, all the ingredients of the mixture being in dry, pulverulent condition, for the purpose set forth.

30 WILLIAM HOSKINS.

In the presence of—

J. G. ANDERSON,  
R. A. RAYMOND.